

Dec. 9, 1969

P. K. ISAACS

3,483,025

FILM COALESCED LATEX IMPREGNATED PAPER AND PROCESS THEREFOR

Filed July 21, 1966



FIG. 1.  
PRIOR ART



FIG. 2.

PHILIP K. ISAACS  
INVENTOR

BY *Francis J. Deep*  
ATTORNEY

1

3,483,025

## FILM COALESCED LATEX IMPREGNATED PAPER AND PROCESS THEREFOR

Philip K. Isaacs, Silver Spring, Md., assignor to W. R. Grace & Co., New York, N.Y., a corporation of Connecticut

Filed July 21, 1966, Ser. No. 566,816  
Int. Cl. C08c 17/18; C08d 13/18

U.S. Cl. 117—155

5 Claims

### ABSTRACT OF THE DISCLOSURE

The invention disclosed is directed to an impregnated paper comprising a cellulosic pulp paper impregnated with coalesced synthetic polymer latex solids with substantially all of the solids being coalesced on the surface of fibers in the paper so that the interior of the fibers are substantially free of latex solids. The paper is impregnated in a process which comprises contacting a synthetic polymer latex with an organic cation/free base organic anion exchange resin and thereafter applying the latex to a cellulosic pulp paper. In a preferred embodiment of the present invention, the latex contains from about 5% to about 70% synthetic polymer and more preferably from about 15% to about 50%.

The present invention relates to a novel and useful product and a process for preparing the product. More particularly, it relates to an impregnated paper and a process for impregnation.

It is known in the art that various latex impregnated papers may be used in the manufacture of pressure sensitive tapes, shoe insoles, artificial leather bases and the like. In the preparation of the latex for paper impregnation, two distinct systems are utilized. The first system utilizes a monomer, water, soap and an initiator which are mixed with heat and pressure. The second system utilizes the polymer, water, a quite large quantity of surfactant and energy which is generally imparted in the form of mixing to disperse the particles. The latex resulting from each of these systems, when applied to a paper, usually results in a bridging of polymer strings between the paper fibers and some actual penetration of the polymer into the fibers. The bridging results in a waste of polymer since the bridges add little, if any, to the strength of the paper. The penetration of the polymer into the fibers also results in a loss of polymer since it actually detracts from the strength of the fibers it has penetrated. In addition, the surface active agent used impair the physical properties of the paper and the resulting tapes are generally not suitable for electrical work since the surfactant increases the conductivity in the finished product. Quite obviously, if a system could be developed which did not utilize a surface active agent and resulted in the fiber being uniformly coated with substantially no bridging or penetration, it would receive widespread acceptance in the art.

It is an object of the present invention to provide a process for preparing an improved latex. A further object is to provide an impregnated cellulosic pulp paper. A still further object is to provide a more uniformly impregnated cellulosic pulp paper. Other objects will become apparent as the description of the invention proceeds.

These objects are accomplished by the present invention which provides a process for impregnating paper which comprises contacting a synthetic polymer latex with an organic cation/free base organic anion exchange resin and thereafter applying the latex to a cellulosic pulp paper.

In a preferred embodiment of the present invention,

2

the latex contains from about 5% to about 70% synthetic polymer and more preferably from about 15% to about 50%.

The present invention also provides an impregnated paper comprising a cellulosic pulp paper impregnated with a coalesced synthetic polymer latex solids with substantially all of the said solids being coalesced on the surface of the fibers in the paper so that the interior of the fibers are substantially free of said latex solids.

In a preferred embodiment of the present invention the impregnated paper contains at least about 20% synthetic polymer latex solids and more preferably from 30 to 100%. In a still more preferred embodiment, the impregnated paper contains from 40 to 60% synthetic polymer latex solids.

The term "latex" is used in its conventional sense to mean a dispersion of solid synthetic polymer particles in water which is capable of forming a film from the dispersion. The synthetic polymers which can be utilized in the latex includes, without limitation, polymers and copolymers of butadiene, isoprene, chloroprene, acrylates, vinyl halides, vinyl esters and the like. Specific examples include the homopolymers polyethyl acrylate, plasticized polyvinyl chloride and the copolymers styrene-butadiene (40%—60%) and styrene-acrylonitrile-butadiene-acrylic acid (35%—14%—50%—1%). Other polymers are likewise suitable.

The expression "organic cation/free base organic anion exchange resin" is used to signify all the conventional organic resins which are utilized for the removal of anions and cations from solutions. The solution may be passed sequentially through the cation exchange resin and then the anion exchange resin (or vice versa) or the resins may be utilized as a mixed bed. Preferably, the anion exchange resin is a strong base resin since a longer contact time is required with the weaker resins. In many instances, the anion exchange resin is furnished in the form of the chloride since it is more stable in this form. In such cases, the chloride should be changed to the free base before being used as the free base does not add ions to the solution. Anion and cation exchange resins are well known in the art and are described in numerous publications, books and patents. A partial list of suitable organic anions and cations resins is given in the "Encyclopedia of Chemical Technology" (1952), volume 8, page 13. Other organic resins are also suitable and may be found in any standard textbook on ion exchange.

The terminology "cellulosic pulp paper" is used to mean any conventional paper such as that made from wood pulp, cotton linters and the like. It also includes paper which contains some synthetic filaments as reinforcement. The term "coalesce" merely signifies that the polymer has been heated sufficiently so as to fuse the particles together.

The invention will now be described by reference to the drawings. In the drawings:

FIGURE 1 is an artist's conception of an enlarged cross sectional view of a sheet of impregnated paper produced in accordance with the prior art; and

FIGURE 2 is an artist's conception of an enlarged cross sectional view of a sheet of impregnated paper produced in accordance with the present invention.

In FIGURE 1 the paper fibers 1 have been penetrated by the polymer 2 and strings of the polymer 3 bridge the individual filaments. The figure demonstrates that the prior art procedures result in a waste of polymer by the bridges being formed and by the polymer penetrating into the fibers.

In FIGURE 2 the paper fibers 4 are substantially uniformly coated with the polymer 5. The figure demonstrates that very little polymer is wasted when the impregnated

paper is made in accordance with the present invention since the polymer is quite uniformly coated onto the filaments.

The following examples are given to illustrate the invention and are not intended to limit it in any manner. All parts are given in parts by weight unless otherwise expressed.

In the following examples, the tests are carried out as follows.

The percent total solids in the latex is determined by accurately weighing a sample of the latex, drying said sample to constant weight and reweighing. The total solids are then calculated from the following formula:

$$\frac{\text{Dry weight}}{\text{wet weight}} \times 100 = \text{percent total solids}$$

Tensile properties, i.e., tensile strength at failure, percent elongation at failure and 1 percent tensile modulus are measured in accord with ASTM-D-412-64T. The copolymer latex is dried in film form (3 mils thick), cut to  $\frac{1}{4}$ " sample strips, placed in the jaws, (2" apart) of a tensile strength tester (Instron, Model TT, available from Instron Engineering Inc., Quincy, Mass.) and separated at a rate of 0.5" per minute and a strain rate of 50% per minute at  $23^{\circ}\text{C}$ . and 50% relative humidity.

The delamination resistance is measured by preparing test specimens which are cut to a length of approximately  $4\frac{1}{2}$  inches in machine direction and a width of approximately 2 inches in the cross direction of the paper. The test specimens are conditioned 48 hours at  $23^{\circ}\text{C}$ . and 50% relative humidity. A 5-inch long strip of rug binding tape is placed on each side of the paper specimen so that the tape extends beyond the ends of the paper. The specimen is then placed on the bottom platen of a press so that approximately 0.5 inch of the tape extends beyond the end of the platen. The specimens are pressed for 30 seconds at  $275^{\circ}\text{F}$ . at a pressure of 5.12 pounds per square inch on the binding tape. The specimens are cooled to room temperature. The specimens are cut in strips approximately 1 inch wide. The two ends of the rug binding tape are pulled apart into two approximately equal plies. The ends of the binding tape are put into the jaws of the Instron tensile tester and, after the first inch of separation, the average force required to separate the paper is recorded at a cross-head speed to 10 inches/min. The delamination resistance of the paper is reported in pounds based on the average values of 3 specimens.

The fold endurance is tested in accordance to the ASTM-D-2167 testing procedure.

The tear strength is tested by the following procedure: Samples are cut into pieces 1 inch by  $4\frac{1}{2}$  inch and conditioned 48 hours prior to testing. A  $\frac{1}{4}$  inch hole is punched in the center of the sample with a punch of the type used to prepare sheets for loose leaf binders. The thickness of the sample is measured to the nearest 0.1 mil on each side of the hole (along the 1 inch dimension of the sample). The fixture is clamped in the upper jaw of an Instron tensile tester. The bottom jaw of the tester is positioned 0.15 inch below the bottom of the test fixtures. The two ends of the sample are clamped in the lower jaw of the Instron tester and the test run (at 10 inches/min.) until the sample tears. The maximum force developed in tearing the sample is recorded. The edge tearing resistance is calculated by dividing the force recorded in grams by the thickness of the sample on the side at which the sample

tore. The tear strength is reported in grams/mil. A fixture comprising a triangular ( $90^{\circ}-45^{\circ}-45^{\circ}$ ) plate, attached by a pivot (at the  $90^{\circ}$  angle) to a  $\frac{1}{4}$  inch rod, is set into the hole in the paper, rod first. The apex of the triangle just touches the paper at the start of the test.

The electrical resistance tests are carried out using the ASTM-D-1000 test procedure.

#### EXAMPLE 1

10 To 1000 grams of a latex containing 50% of solids (40% styrene-60% butadiene copolymer) is mixed with 200 grams of a mixed bed ion exchange resin and 200 grams of water. The cation portion of the mixed bed is a styrene/divinyl benzene sulfonic acid resin. The anion portion of the bed is a quaternary base of a styrene/divinyl benzene copolymer having a tetramethylamino-methyl group attached to the benzene rings (free base form of resin). The resin is described in J. A. Kitchener "Ion Exchange Resin," Methuen and Co. Ltd., London (1957), page 17. The mixture is stirred at  $50^{\circ}\text{C}$ . for 3 hours and then filtered to remove the resin. Ash content shown that over 95% of the ions are removed. The final solids content is 35 to 40%. A standard size sheet ( $8\frac{1}{2}$  inch by 11 inches) of cotton linters paper (12 mils thick) is impregnated with the latex by dipping the base into the latex to give an impregnated paper having 40% polymer solids (dry weight). The sheet is air dried at room temperature.

20 When the impregnated sheet is examined under a high powered microscope, it can be seen that the fibers have been quite uniformly coated with the latex solids with the substantial absence of any strings or bridges connecting the fibers. By taking  $\frac{1}{2}$  of the paper sheet before 30 drying, the latex on the exterior of the sheet can be removed by washing with water leaving only that latex which has penetrated into the fibers. A comparison of the weight of the washed dried sheet with the weight of the original sheet, shows that substantially no latex has penetrated into the fibers. In contrast, when a control latex is carried through the same procedure without the treatment, a great deal of bridging takes place between the fibers of the paper. Also, by the removal of the latex solids from the sheet, it can be determined that about 15% of the latex solids has penetrated the interior of the fibers.

45

#### EXAMPLES 2-5

The procedure of Example 1 is repeated utilizing a commercial mixed bed anion and cation exchange resin. The commercial resin wherein the cation exchange resin consists of a sulfonated copolymer of styrene and divinyl benzene combined with an anion exchange resin of a styrene-divinyl benzene copolymer matrix containing a quaternized base of dimethyl amino methacrylate. "Illcoway TM-1" is marketed by the Illinois Water Treatment Company. In Example 2, the latex polymer is the same as that utilized in Example 1. In Example 3 the latex polymer is a copolymer containing 35% styrene, 14% acrylonitrile, 50% butadiene and 1% acrylic acid. In Example 4 polyethyl acrylate is utilized and Example 5 uses a plasticized vinyl chloride marketed under the name of "Geon 450X23" (Goodrich Chemical Company). In each example the properties resulting from the deionized latex are compared to those of the same latex without such treatment. The properties for the products are given 50 in the following table:

| Example | Tensile        | Delamination          |            | Fold Endurance | Tear Strength |
|---------|----------------|-----------------------|------------|----------------|---------------|
|         |                | Elongation Resistance | Resistance |                |               |
| 2-----  | Untreated..... | 1,000                 | 14         | 0.44           | -----         |
|         | Deionized..... | 1,100                 | 17         | 0.53           | 0.50          |
| 3-----  | Untreated..... | 900                   | 11         | 0.9            | 0.47          |
|         | Deionized..... | 1,000                 | 13         | 1.2            | 220           |
| 4-----  | Untreated..... | 720                   | 20         | 0.77           | 800           |
|         | Deionized..... | 740                   | 32         | 1.07           | 0.45          |
| 5-----  | Untreated..... | 1,100                 | 19         | 0.71           | 0.63          |
|         | Deionized..... | 1,200                 | 19         | 1.35           | 0.37          |

When the impregnated papers prepared in accordance with the present invention are examined under the microscope the results are substantially the same as in Example 1. When the latex is removed from the product as in Example 1, it shows there is substantially no penetration of the latex into the fibers of the paper just as in Example 1.

#### EXAMPLE 6

The procedure of Example 4 is repeated employing a latex having a solids content of 60%. After deionization, however, the latex is concentrated to a solids content of 40%. After impregnating the sheet, the product has substantially the same properties as that produced in Example 4.

#### EXAMPLES 7-11

The first part of the procedure of Example 3 is repeated using 150 grams of water rather than 200 grams of water. The resulting latex contains 40% by weight of synthetic polymer solids. In Example 7 the resulting latex is diluted to 5% solids to give an uptake on the paper of 6%. In Example 8 the resulting mixture is diluted to 10% solids to give an uptake on the paper of 20%. In Example 9 the resulting mixture is diluted to 20% solids to give an uptake on the paper of 40%. In Example 10 the resulting mixture is diluted to 30% solids to give an uptake on the paper of 60% and in Example 11 the resulting mixture 40% solids is used to give an uptake on the paper of 90%. The properties of the resulting impregnated paper are given in the following table.

| Example                | Percent Polymer | Tensile | Delamination resistance | Fold endurance | Tear strength |
|------------------------|-----------------|---------|-------------------------|----------------|---------------|
| 7..... Untreated.....  | 6               | 604     | 0.30                    | 18             | 0.28          |
| 7..... Deionized.....  | 6               | 676     | 0.40                    | 20             | 0.27          |
| 8..... Untreated.....  | 20              | 738     | 0.58                    | 68             | 0.31          |
| 8..... Deionized.....  | 20              | 904     | 0.50                    | 130            | 0.38          |
| 9..... Untreated.....  | 40              | 909     | 0.94                    | 223            | 0.47          |
| 9..... Deionized.....  | 40              | 1022    | 1.020                   | 795            | 0.45          |
| 10..... Untreated..... | 60              | 971     | 1.40                    | 536            | 0.57          |
| 10..... Deionized..... | 60              | 1240    | 1.70                    | 1968           | 0.64          |
| 11..... Untreated..... | 90              | 1046    | 1.93                    | 412            | 0.63          |
| 11..... Deionized..... | 90              | 1200    | 2.58                    | 1422           | 0.74          |

#### EXAMPLE 12

In order to show the advantages in electrical properties with the paper produced in accordance with the present invention, the process of Example 3 is repeated employing a crepe paper. For comparison purposes, the electrical resistivity is given for the paper, the untreated resin impregnated paper and the deionized resin impregnated paper. The properties are given in the table below:

| Latex          | Paper      | Percent polymer in paper | Electrical resistivity at 90% RH (ASTM-D-1000) megohms. |
|----------------|------------|--------------------------|---------------------------------------------------------|
| Untreated..... | Crepe..... | 0                        | 12                                                      |
| Do.....        | do.....    | 40                       | 2                                                       |
| Deionized..... | do.....    | 40                       | 26                                                      |

While in the above examples unmodified latex systems are utilized, it is obvious that latex systems containing anti-oxidants, fillers, pigments, oils, thickeners and the like can be employed.

Many equivalent modifications will be apparent to those skilled in the art from a reading of the foregoing without a departure from the inventive concept.

What is claimed is:

1. A process for coating the surface of fibers of paper which comprises, applying a synthetic polymer latex containing from about 5% to about 70% synthetic polymer having over 95% of ions removed therefrom by contacting with an organic cation/free base organic anion exchanged resin, thereafter applying the said latex to a cellulosic pulp paper, and drying the impregnated paper sufficiently so as to substantially coalesce the synthetic polymer on the surface of the fibers of the paper whereby the interior of the fibers is substantially free of said synthetic polymer.

2. The process of claim 1 wherein the latex contains from about 15% to about 50% synthetic polymer.

3. A fiber-coated paper which comprises a cellulosic pulp paper fiber-coated with at least 20%, based on the weight of the paper, of coalesced synthetic polymer latex solids having over 95% of ions removed therefrom by contacting with an organic cation/free base organic anion exchange resin, substantially all of the said latex solids being coalesced on the surface of the fibers of the paper whereby the interior of the fibers is substantially free of said synthetic polymer.

4. The fiber-coated paper of claim 3 wherein the synthetic polymer latex solids are present in an amount from about 30% to about 100% based on the weight of the paper.

5. The fiber-coated paper of claim 3 wherein the synthetic polymer latex solids are present in an amount from

about 40% to about 60% based on the weight of the paper.

#### References Cited

##### UNITED STATES PATENTS

|    |           |         |                 |           |
|----|-----------|---------|-----------------|-----------|
| 45 | 3,262,811 | 7/1966  | Sellet          | 117-155 X |
|    | 2,912,349 | 11/1959 | Videen et al.   | 117-161   |
|    | 2,912,350 | 11/1959 | Videen et al.   | 117-161   |
|    | 2,961,417 | 11/1960 | Small           | 260-2.1   |
|    | 3,017,295 | 1/1962  | Otterson et al. | 117-155   |
|    | 3,041,292 | 6/1962  | Hatch           | 260-2.1   |
|    | 3,114,485 | 11/1963 | Kunin           | 210-38 X  |
|    | 3,205,184 | 9/1965  | Hatch           | 210-38 X  |
|    | 3,300,416 | 1/1967  | Hatch           | 260-2.1   |
|    | 3,303,155 | 2/1967  | Peterson et al. | 117-155 X |
| 50 | 3,332,890 | 7/1967  | Hatch           | 260-2.1   |
|    | 3,335,100 | 8/1967  | Geyer           | 117-201 X |

##### FOREIGN PATENTS

|    |           |        |          |
|----|-----------|--------|----------|
| 60 | 1,131,013 | 6/1962 | Germany. |
|----|-----------|--------|----------|

WILLIAM D. MARTIN, Primary Examiner

M. R. LUSIGNAN, Assistant Examiner